

# UNITED STATES PATENT OFFICE.

FRANK H. WELSH, OF RICHMOND, CALIFORNIA.

## SURFACING MIXTURE FOR PAVEMENTS AND OTHER STRUCTURES.

1,209,238.

Specification of Letters Patent. Patented Dec. 19, 1916.

No Drawing.

Application filed February 21, 1916. Serial No. 79,477.

To all whom it may concern:

Be it known that I, FRANK H. WELSH, a citizen of the United States, residing at Richmond, in the county of Contra Costa and State of California, have invented certain new and useful Improvements in Surfacing Mixtures for Pavements and other Structures, of which the following is a specification.

10 My invention relates to compositions of matter of the asphalt type.

The primary object of my invention is to provide a composition of matter well adapted for use as a surfacing mixture for pavements of roads, old or new, sidewalks, cellars and other structures. It may also be used for waterproofing roofs, sewer and water pipe, brick structures, and reservoirs, and for damp-proofing foundations. Finally, 20 it may be used also in the construction of complete pavements, and as a binder or filler in the construction of roads, streets and sidewalks of all classes and specifications.

My composition of matter consists essentially of the asphalt residuum of steam-distilled crude-petroleum as I shall hereinafter describe, and a special crude petroleum air-treated product which I shall fully describe, the two being mixed under conditions of 30 temperature and in the proportions substantially as hereinafter specified. To these essential ingredients may be added, if necessary, as, for example, to harden or toughen the mixture, a small amount of carbonate of lime.

The asphalt used in my composition is the product of the following preparation, and may, for convenience, be termed steam distilled asphalt. Crude oil is subjected to the 40 well known process of steam distillation, by which all the lighter oils are fractioned off and removed either in one continuous stream from which the several cuts are made to define gasoline, engine distillate, burning oil 45 or kerosene, etc., or in several operations, to more thoroughly remove these fractions, so that a residue remains, which has the required ductility and penetration for a particular brand or purpose. This residue is 50 then drawn off, run through coolers to reduce its temperature and finally is run into barrels and stored or sold as asphalt of a certain degree of penetration and ductility. This is the asphalt of commerce and from it, 55 as has been stated, all the lighter oils or frac-

tions of the original crude oil have been removed.

The special petroleum product which forms the other essential ingredient of my composition is the result of the following well known preparation, and may conveniently be termed an air-blown petroleum product. Crude oil is subjected in a still to heat and is treated with air blown into it under pressure, the temperature and duration being such as to gradually thicken the mass until it reaches the required penetration and ductility. During this operation the lighter oils are not removed. The batch or mix is left in the still until it is reduced to its proper penetration and ductility, and it is then drawn off, cooled and barreled, as in the case of the commercial asphalt. This air-blown petroleum product comes from the still as a tough, rubbery mass, containing nearly all the ingredients of the original crude oil, but changed in chemical combination. It contains more carbon than does the commercial asphalt, or rather, the air blowing separates the carbon more than does the steam blowing.

Commercial asphalt in itself becomes dry and hard with use and is brittle. The air-blown petroleum product has the toughness and resistance to abrasion that asphalt lacks, but it has so much free carbon that it is lacking in the cohesion required for ductility. The proper mixing of the two gives a composition which has all the plastic consistency of the asphalt, added to the tough, rubbery, wearing qualities of the air-blown product, and the oils present keep the mixture from carbonizing and thus losing cohesiveness, said mixture having the required resistance to abrasion and a resiliency not possible with asphalt alone.

Having now described the essential ingredients of my composition, the following statement of their mixing, both as to temperature conditions and proportions will be understood. This statement is, however, given only as one example of the mixing, for the temperature and proportions will vary according to climatic conditions prevalent in the locality where the composition is to be used, such variation being dependent upon the results sought, as to hardness, toughness, durability, etc., which desiderata are all well known to those skilled in the art and are within the common knowledge of

and may be carried out by practitioners, when once informed, as by this specification and example, of the advantageous result which follows the production of my mixture.

5 The mixture is made as follows: steam distilled crude petroleum residuum asphalt 70% by weight, crude petroleum air-blown product 20% by weight. To which may be added carbonate of lime 10% by weight.

10 These ingredients are mixed under a temperature of not less than 350 degrees Fahr.

In practice, I prefer to use asphalt of 150 degrees penetration, D. C. standard. The air-blown product is generally known on the 15 market as petroelastic cement, and the kind I prefer to use is known commercially as No. XXX-50.

The mixture should be used at a temperature of not less than 350 degrees Fahr., and 20 is applied as a surfacer by means of pressure or gravity atomizers, sprayers, squilgees, buckets, pails, etc.

I am aware of asphaltic cements composed of residual bitumens and a relatively small 25 percentage, not exceeding 10% of a blown oil flux, the latter being used to soften the bitumen. These cements are particularly

affected by temperature changes, and they are, therefore, used only in a mixture with a suitable aggregate, the mixture being carefully prepared prior to laying on the street and as cautiously used lest it be too soft or too hard. Without this aggregate they are unsuitable for paving purposes, and cannot be used for surfacing.

30

35

I claim:—

An asphaltic surfacing composition devoid of aggregate and comprising a mixture of steam-distilled, crude-petroleum residuum asphalt from which the volatile constituents have been removed, and substantially 20% by weight of a product derived from crude petroleum by treating it while under heat with air under pressure, without removing its volatile constituents, substantially as described.

40

45

In testimony whereof I have signed my name to this specification in the presence of two subscribing witnesses:

FRANK H. WELSH.

Witnesses:

W.M. F. BOOTH,  
D. B. RICHARDS.